

F. W. ADAMS.

PROCESS OF NAPPING AND SATURATING FELT AND PRODUCT THEREOF.

APPLICATION FILED JUNE 29, 1918.

**1,311,862.**

Patented July 29, 1919.



INVENTOR

*Floyd W. Adams*

BY

*Chas. W. Mortimer*

ATTORNEY

# UNITED STATES PATENT OFFICE.

FLOYD W. ADAMS, OF HUDSON HEIGHTS, NEW JERSEY, ASSIGNOR TO THE BARRETT COMPANY, A CORPORATION OF NEW JERSEY.

## PROCESS OF NAPPING AND SATURATING FELT, AND PRODUCT THEREOF.

1,311,862.

Specification of Letters Patent.

Patented July 29, 1919.

Application filed June 29, 1918. Serial No. 242,611.

*To all whom it may concern:*

Be it known that I, FLOYD W. ADAMS, a citizen of the United States, residing at Hudson Heights, in the county of Bergen 5 and State of New Jersey, have invented certain new and useful Improvements in Processes of Napping and Saturating Felt, and Product Thereof, of which the following is a specification.

10 This invention relates to a new and useful construction material and the method of producing the same. It is directed more particularly to the saturation of felts or paper which are to be used as building materials, 15 and is designed to enable a more thorough saturation or impregnation of the felt or paper base than has been possible with the usual methods of saturation.

In practising this invention I may take 20 an ordinary sheet of felt or paper such as is used for making roofing material, etc. and nap or pick the surface thereof either at the felt-making mill or just prior to saturating it in order to produce a surface which will 25 more readily absorb a saturant. The felt or paper having the napped surface on one or both sides may be immersed in a liquid bath of the usual saturating or waterproofing materials such as tar, oil, or any suitable water- 30 proofing materials already in use for such purposes. The interior of the felt or paper which is unaffected by the napping process will absorb the customary amount of saturant during the saturating operation, but 35 the napped surface, being more loose or less compact, will mechanically carry a correspondingly larger amount of the saturant, a portion of which will be gradually absorbed by the denser interior of the felt or paper 40 with the lapse of time after the sheet has passed through the saturating bath.

The invention will be understood by reference to the accompanying drawing in which the figures represent somewhat dia- 45 grammatically a sheet being napped and passed through a bath of saturating material.

In this drawing the reference character 1 represents a roll of felt or paper which has 50 been produced in the ordinary way as, for example, on a paper-making machine having a foraminous cylinder. In making this sheet the usual paper-making stock, such as rag or wood fibers, may be used. After 55 the sheet has been made and dried in the customary manner it is rolled up into the

roll 1 from which it may be unrolled in carrying out the process and making the product of the present invention.

The sheet 2 is unwound from the roll 1 60 and passes in proximity to a napping device such as is represented by the cylinders 3 having pickers 4 thereon. These cylinders may all be driven in the same direction, or some of them, as indicated at 3' may be driven 65 in the opposite direction by any suitable means, not shown. It is obvious that the number and disposition of these cylinders may be varied to suit the circumstances so that only one or both sides of the sheet will 70 be napped and the degree and depth of the napping may be varied within wide limits. The particular sort of napping device is im- 75 material, the desideratum being that the surface or surfaces of the sheet should be napped to some depth so that the outside fibers will be loosened up to a considerable extent and thereby become more porous and absorbent for the saturant.

After the surface of the sheet 2 has been 80 napped as indicated at 5, the napped sheet may be passed through a liquid bath 6 of waterproofing material such as oil, tar, creosote, asphalt, etc. If necessary, this bath may be heated in any convenient or suit- 85 able manner to render the saturant more fluid.

As the sheet 2 passes through the saturant 6 the interior of the same which has been unaffected by the napping operation absorbs 90 a certain amount of saturant, while the outside napped portion, being loose and less dense, mechanically carries a proportionately larger amount of the saturant. This excess may be regarded as a layer or 95 layers 7 of saturant on the outside of the sheet, having the fibers, which constitute the napping, interspersed therethrough and being prevented from dripping off by means of these fibers. The saturated sheet may 100 then be rolled up into the roll 8 where a portion of the layer 7 of saturant is gradually absorbed into the more dense portions of the sheet. In this way a larger amount of saturant can be introduced into a sheet 105 of felt than has been hitherto possible with the usual saturating processes. If desired the sheet may be rolled up while the saturant is still warm or the roll may be kept heated by outside heating agencies in order to pro- 110 mote the absorption whenever found necessary.

The napping of sheets makes them mechanically weaker, but the increase in the amount of saturation which is obtainable by napping serves to increase the strength thereby rendering them, after saturation, approximately as strong as the saturated unnaped sheet. Tests have shown that with some saturants, such as asphalt, the saturated napped sheets were actually stronger than the unnaped saturated sheets.

10 The grade of a saturated sheet is partially determined by its weight, so that an increase of the saturant serves to increase its value, and improve its waterproofing qualities.

15 After the sheets have been saturated, they may be used for the same purposes heretofore available for the usual saturated sheets. A useful and salable product may, however, be produced merely by napping the

20 sheets, made from paper-making stock, without saturating the same. That is, the sheets as they come from the napping device may be removed without being saturated, and such napped unsaturated sheets are within

25 the scope of this invention. I do not claim the production of napped woolen goods such as blankets, but what I do claim and desire to secure by Letters Patent is:

1. As an article of manufacture, a sheet of napped felt saturated with waterproofing material.

2. As an article of manufacture, a sheet of napped paper saturated with asphalt.

3. The process of producing a construction material which comprises the steps of napping the surface of a building felt and applying waterproofing material to the napped felt.

4. The process of producing a construction material which comprises the steps of

napping the surface of a building felt and applying waterproofing material to the napped felt and rolling the treated sheet up so that the waterproofing material in the napped portion is partially absorbed into the interior.

45

5. The process which comprises saturating the surface of a napped sheet of paper-making material with waterproofing material and subsequently causing the saturant to penetrate the interior of the sheet.

50

6. The process of saturating a sheet of napped felt which comprises the steps of introducing saturant into the interior of the felt, applying a layer of excess saturant to the surface of the sheet and subsequently causing the excess saturant to become absorbed into the interior.

55

7. The process of producing a construction material which comprises treating the surface of a sheet of paper-making material so as to render said surface more porous than the interior of said sheet and saturating said sheet with waterproofing material.

60

8. The process of producing a construction material which comprises picking the surface of a sheet of paper-making material so as to render said surface more readily absorbent of waterproofing material, and saturating said sheet with waterproofing material.

65

9. As an article of manufacture, a sheet of felt having its surface treated so that the capacity of said surface for absorbing waterproofing material is proportionately greater than the interior of said sheet, said sheet being saturated with waterproofing material.

70

In testimony whereof I affix my signature.

FLOYD W. ADAMS.